

3,411,917

SENSITIZATION OF SILVER HALIDE EMULSIONS  
WITH DIRECT ELECTRICAL CURRENT  
John Figueras, Rochester, N.Y., assignor to Eastman  
Kodak Company, Rochester, N.Y., a corporation of  
New Jersey  
No Drawing. Filed Apr. 29, 1965, Ser. No. 451,992  
9 Claims. (Cl. 96—107)

## ABSTRACT OF THE DISCLOSURE

Photographic silver halide emulsions are sensitized by passing a direct electrical current having a voltage of 3-12 volts therethrough. The sensitization treatment increases the speed of the photographic emulsion. It can be used in conjunction with other chemical sensitizing treatments such as, for example, sulfur-type and noble metal sensitization. The electrolysis treatment can be performed either before or after the other sensitizing treatments. Especially useful results have been obtained where the treatment was carried out following the other sensitizing operations.

This invention relates to photography, and more particularly, to a new method for the reduction sensitization of photographic silver halide emulsions.

It is known that the sensitivity of silver halide emulsions can be increased by several methods, including spectral sensitization and chemical sensitization. In spectral sensitization, the optical range of sensitivity, is increased, while in chemical sensitization, the overall sensitivity of a photographic emulsion is improved. The present invention is concerned primarily with the latter type of sensitization.

Among the common forms of photographic chemical sensitizations there are sulfur-type sensitization, noble metal sensitization, and reduction sensitization. The first involves treatment of silver halide emulsions with compounds of the sulfur family and is believed to result in the formation of sensitivity specks in or on the silver halide grain; the second comprises the addition of a noble metal salt or compound with the possible formation of noble metal nuclei in or on the silver halide grain; the third, i.e., reduction sensitization, has been performed by the addition of compounds having a sufficiently strong capacity to reduce silver halide to metallic silver. Reduction sensitization is extremely useful since it can be additive to the former two forms of chemical sensitization.

It is, accordingly, an object of this invention to provide an improved method of reduction sensitizing photographic silver halide emulsions. Still another object of my invention is to provide a new method of reduction sensitization which is relatively easy to apply and which requires no chemical treatment. It is a further object of my invention to provide a method of reduction sensitization which obviates the critical features inherent in chemical procedures of reduction sensitization. Another object of this invention is to further increase the speed of sulfur-type and/or noble metal sensitized silver halide emulsions by the reduction sensitizing method disclosed in this invention. It is still a further object to provide high speed reduction-sensitized emulsions with low fogging propensity as well as improved keeping stability. It is an object of my invention to provide an improved nonchemical method of reduction sensitization of photographic silver halide emulsions by electrolytic means. Other objects of my invention will appear herein.

In its broadest aspects, the above objects are accom-

plished by passing D.C. electric current through an aqueous silver halide photographic emulsion. For example, through an aqueous silver halide photographic emulsion is passed by means of inert electrodes a direct electrical current. I have found that either carbon or silver electrodes are eminently suitable for use in this connection. Although any voltage which will supply sufficient potential to force the electric current through the emulsion can be used, ordinarily a value within the range of 3-12 volts would be employed for an electrode spacing of 3 inches. Variation of treating conditions is possible as may be selected by the individual operator in any particular situation. For instance the emulsion may be conveniently sensitized in accordance with the invention while subjected to stirring or other agitation and at a temperature assuring good liquidity for example 40° C.

The present invention makes possible a more advantageous combination of reduction sensitization, noble metal sensitization and sulfur-type sensitization, while maintaining, within controllable limits, fog and stability of the treated emulsions.

Where the new reduction sensitizing procedure of my invention is used in conjunction with other chemical sensitizing, for example, sulfur-type and noble metal sensitization, the electrolysis can optionally be performed either before or after the other sensitizing treatments. Especially useful results have been obtained where the treatment was performed following the other sensitizing operations.

My electrical method of reduction sensitizing photographic silver halide emulsions can be used with emulsions having a gelatin vehicle. It operates advantageously with emulsions containing a mixture of gelatin and one or more other hydrophilic colloids such as polyvinyl alcohol, gum arabic, ethyl acrylate-acrylic acid copolymer, butyl acrylate-acrylic acid copolymer, etc.

My invention is not confined to any particular sulfur-type sensitizer or group of sulfur-type sensitizers, although the following are particularly useful in practicing my invention: allylisothiourea, allylthiourea, allylisothiocyanate, phenylisothiocyanate, phenylthiourea, sodium thiosulfate, thiocarbanilide, thiourea, thiosemicarbazide, thioacetamide, thioformamide, thiobarbituric acid, etc. Such well known sensitizers have been previously described in Sheppard U.S. Patent 1,574,944, issued Mar. 2, 1926; Sheppard et al. U.S. Patent 1,623,499, issued Apr. 5, 1927; Sheppard et al. U.S. Patent 2,410,689, issued Nov. 5, 1946, etc.

Noble metal salts or compounds useful in sensitizing emulsions are also well known to those skilled in the art and comprise auric trichloride, sodium chloroaurate, potassium chloroaurite, potassium bromaurite, potassium iodoaurite, potassium iodoaurate, potassium aurithiocyanate, potassium aurichloride, auric sulfate, sodium auric chloride, potassium auric bromide, sodium auric bromide, alkali metal aurous thiosulfate, alkali metal aurous sulfite, thiourea-auric chloride complex, auric chloride-3-ethyl-5-[(3-ethyl)-2-(3H)-benzoxazolylidene)ethylidene]rhodanine addition product (e.g., Damschroder et al. U.S. Patent 2,642,361, issued June 16, 1953), etc. Typical gold sensitizers are described in Waller et al. U.S. Patent 2,399,083, issued Apr. 23, 1946.

The following examples illustrate my invention and are not limiting thereof:

## EXAMPLE 1

To 317 grams of optimally finished sulfur-gold sensitized emulsion containing 0.10 mole of silver halide and 24.5 grams of gelatin, was added 0.20 gram of 4-hydroxy-6-methyl-1,3,3a,7-tetraazaindene antifoggant in 6.0 cc. of water. The pH of the emulsion was adjusted to 6.0 and

silver rod electrodes of about  $\frac{1}{4}$  inch in diameter and 3 inches in length were immersed in the emulsion. Current was passed through the emulsion for 3 minutes by means of the electrodes. The current source was two 6-volt dry cells wired in series which provided a current from approximately 80 to 120 ma. This corresponded to a current density at the electrodes of about 10 ma./cm.<sup>2</sup>. After electrolysis, the emulsion pH was adjusted to 6.4 and the emulsion pAg was adjusted to 8.3. Water and additional gelatin were added and the emulsion was coated on transparent film support at a silver coverage of 540 mg./ft.<sup>2</sup> and a gelatin coverage of 1225 mg./ft.<sup>2</sup>. The emulsion coating was dried, sensitometrically exposed in an Eastman 1B sensitometer, and developed for 5 minutes at a temperature of 68° F. in a developing solution of the following composition:

|                                            |       |      |
|--------------------------------------------|-------|------|
| Water -----                                | ml    | 500  |
| Methyl-p-aminophenol -----                 | gm    | 2.5  |
| Sodium sulfite, des. -----                 | gm    | 30.0 |
| Hydroquinone -----                         | gm    | 2.5  |
| Sodium metaborate, 8H <sub>2</sub> O ----- | gm    | 10.0 |
| Potassium bromide -----                    | gm    | 0.5  |
| Water to make -----                        | liter | 1.0  |

A similar coating was made of unelectrolyzed emulsion.

After development, the film samples were fixed, washed, and dried in the conventional manner.

The sensitometric results were as follows:

|                              | Rel. Speed | Gamma | Fog  |
|------------------------------|------------|-------|------|
| Nonelectrolyzed coating----- | 100        | 2.40  | 0.04 |
| Electrolyzed coating-----    | 182        | 2.20  | 0.08 |

#### EXAMPLE 2

A fine grain negative silver bromoiodide gelatin emulsion sample, optimally finished and chemically sensitized to its maximum speed with gold and sulfur sensitizers was electrolyzed and processed according to procedures described under Example 1. An emulsion sample identical to the above, but not electrolyzed, was coated and processed to serve as a control. The sensitometric results were as follows:

|                              | Rel. Speed | Fog  |
|------------------------------|------------|------|
| Nonelectrolyzed coating----- | 100        | 0.10 |
| Electrolyzed coating-----    | 145        | 0.23 |

The electrolysis increased the fog level of this particular emulsion used; but after allowance is made for this fog, it is seen that electrolysis has increased the emulsion speed by approximately 50%. That the occurrence of fog is not a necessary feature of the electrolytic process of my invention is shown in the following example.

#### EXAMPLE 3

The same type of emulsion as described under Example 2 was electrolyzed in the presence of 2.0 gm./silver mole of 4-hydroxy-6-methyl-1,3,3a,7-tetraazaindene antifoggant and compared with an emulsion sample electrolyzed without containing the above addendum.

|                                                                                  | Rel. Speed | Fog  |
|----------------------------------------------------------------------------------|------------|------|
| Sample without 4-hydroxy-6-methyl-1,3,3a,7-tetraazaindene-----                   | 100        | 0.23 |
| Sample with 2 gm./silver mole of 4-hydroxy-6-methyl-1,3,3a,7-tetraazaindene----- | 110        | 0.12 |

This table shows that azaindene antifoggants keep the fog from increasing when they are present during reduction sensitizing by electrolysis.

Similar results are obtained with other types of azaindenes such as those described in Heimbach and Kelly U.S. Patents 2,444,605, and 2,444,606, issued July 6, 1948; Heimbach U.S. Patents 2,444,607, issued July 6, 1948, and 2,450,397, issued Sept. 28, 1948; Heimbach and Clark U.S. Patent 2,716,062, issued Aug. 23, 1955; Allen and Reynolds U.S. Patents 2,713,541, issued July 19, 1955, and 2,743,181, issued Apr. 24, 1956; Carroll and Beach U.S. Patent 2,716,062, issued Aug. 23, 1955; Allen and Beilfuss U.S. Patent 2,735,769, issued Feb. 21, 1956; Reynolds and Sagal U.S. Patent 2,756,147, issued July 24, 1956; Allen and Sagura U.S. Patent 2,772,164, issued Nov. 27, 1956, and those disclosed by Birr in "Z. wiss Phot.", Vol. 47, 1952, pages 2-28.

The new method of reduction sensitization of my invention is also applicable in the presence within an emulsion of other known stabilizing compounds such as the triazoles of Heimbach and Kelly U.S. Patent 2,444,608, issued July 6, 1948; the zinc and cadmium salts of Jones U.S. Patent 2,839,405, issued June 17, 1958; the carboxymethylmercapto compounds of Murray, Reynolds and Van Allan U.S. Patent 2,819,965, issued Jan. 14, 1958; and the disulfides of Kodak Belgian Patent 569,317, issued July 31, 1958.

Examples 4, 5 and 6 show respectively the electrolysis effect on emulsions which (a) bear no prior chemical sensitization, (b) are sulfur sensitized, and (c) are sulfur-gold sensitized.

#### EXAMPLE 4

Medium grain silver bromoiodide gelatin emulsion containing 2 gm./silver mole of 4-hydroxy-6-methyl-1,3,3a,7-tetraazaindene but having no chemical sensitization was subjected to a direct current electrolysis as described in Example 1. The photographic product obtained was tested in the manner previously described with the following results:

|                             | Rel. Speed | Fog  |
|-----------------------------|------------|------|
| Nonelectrolyzed sample----- | 100        | 0.09 |
| Electrolyzed sample-----    | 162        | 0.10 |

#### EXAMPLE 5

Sulfur sensitized coarse-grain silver bromoiodide gelatin emulsion containing no 4-hydroxy-6-methyl-1,3,3a,7-tetraazaindene was employed as the emulsion in a run similar to that of Example 1. The following results were obtained:

|                             | Rel. Speed | Fog  |
|-----------------------------|------------|------|
| Nonelectrolyzed sample----- | 100        | 0.06 |
| Electrolyzed sample-----    | 132        | 0.08 |

#### EXAMPLE 6

Sulfur-gold and selenium-gold sensitized medium-grain silver bromoiodide gelatin emulsions containing 2 gm./silver mole of 4-hydroxy-6-methyl-1,3,3a,7-tetraazaindene were electrolyzed as described in Example 1. The results obtained were as follows:

|                                  | Non-Electrolyzed |       |      | Electrolyzed |       |      |
|----------------------------------|------------------|-------|------|--------------|-------|------|
|                                  | Speed            | Gamma | Fog  | Speed        | Gamma | Fog  |
| Sulfur-gold sensitization-----   | 100              | 2.64  | 0.06 | 145          | 2.56  | 0.08 |
| Selenium-gold sensitization----- | 100              | 2.60  | 0.20 | 162          | 2.60  | 0.22 |

Photographic speed increasing compounds can be used in emulsions which are reduction sensitized by the electrolytic method of my invention. Such compounds can be of the quaternary ammonium type of Carroll U.S. Patent 2,271,623, issued Feb. 3, 1942; Carroll and Allen U.S. Patent 2,288,226, issued June 30, 1942; and Carroll and Spence U.S. Patent 2,334,864, issued Nov. 23, 1943; or the polyethylene glycol type of Carroll and Beach U.S. Patent 2,708,162, issued May 10, 1955; or the quaternary ammonium salts and polyethylene glycols of Piper U.S. Patent 2,886,437, issued May 12, 1959; as well as the thiopolymers of Graham and Sagal U.S. Patent 3,046,129, issued July 24, 1962, and Dann and Chechak U.S. Patent 3,046,134, issued July 24, 1962.

In experiments performed with emulsions containing speed increasing compounds mentioned above, significant increases in speed were shown by the electrolyzed emulsion over the control, and the speed effects of the addenda were approximately additive to the speed gained from electrolysis.

The electrolytic procedure of my invention is also applicable when a higher degree of reduction even up to complete fogging of a silver halide emulsion is desired, as for example in the preparation of photographic direct positive materials. The reduction of silver halide grains for the preparation of direct positive materials is commonly achieved either by the addition to a photographic negative emulsion of compounds such as formaldehyde (see Kendall and Hill, U.S. Patent 2,541,472) or stannous chloride or by exposing the emulsion to high intensity light radiation.

Accordingly, my invention also provides a new method for reduction fogging of photographic emulsions for use as direct positive materials. This method consists generally of subjecting an emulsion to electrolysis as described above, in which electrolytic potential, time of treatment, and other conditions are selected in order to achieve the degree of reduction desired. The practice of my invention envisions the combination of conventional treatment by chemical addenda with electrolytic reduction to achieve the degree of reduction needed in a particular circumstance.

In the practice of my invention, electrical potentials ranging from 3 to 12 volts have been applied. Higher or lower potentials can be used depending on the internal resistance and the current flow desired. Potentials ranging from approximately 1½ volts to at least 12 volts are considered useful, depending on the operating conditions and desired extent of emulsion reduction.

The speed increase from electrolysis appears to be the result of an improvement in granularity efficiency rather than a development effect. This is shown by two pieces of evidence. First, the sensitometric speed gain from electrolysis is independent of the degree of development. Secondly, the speed obtained from electrolysis is not accompanied by any increase in the granularity of the film.

The invention has been described in considerable detail with particular reference to certain preferred embodiments thereof, but it will be understood that variations and modifications can be effected within the spirit and scope of the invention as described hereinabove, and as defined in the appended claims.

I claim:

1. A method of sensitizing an aqueous silver halide photographic emulsion which comprises passing a direct electrical current having a voltage of 3-12 volts therethrough.

2. A method of sensitizing a sulfur-sensitized aqueous silver halide photographic emulsion which comprises passing a direct electrical current having a voltage of 3-12 volts therethrough.

3. A method of sensitizing a noble-metal sensitized aqueous silver halide photographic emulsion which comprises passing a direct electrical current having a voltage of 3-12 volts therethrough.

4. A method of sensitizing an aqueous silver halide photographic emulsion, which has been chemically sensitized with a labile element of the sulfur family and a noble metal compound, which comprises passing a direct electrical current having a voltage of 3-12 volts therethrough.

5. A method of sensitizing a selenium sensitized aqueous silver halide photographic emulsion which comprises passing a direct electrical current having a voltage of 3-12 volts therethrough.

6. A method of sensitizing an aqueous silver halide photographic emulsion containing an antifoggant which comprises passing a direct electrical current having a voltage of 3-12 volts therethrough.

7. A method of sensitizing an aqueous silver halide photographic emulsion which comprises passing therethrough a direct electrical current having a voltage of 3-12 volts using silver electrodes.

8. A method of sensitizing an aqueous silver halide photographic emulsion which comprises passing therethrough a direct electrical current having a voltage of 3-12 volts using carbon electrodes.

9. A method of producing a fogged aqueous silver halide photographic emulsion useful in the production of photographic direct positive materials which comprises passing a direct electrical current having a voltage of 3-12 volts through an aqueous silver halide photographic emulsion until said fogged aqueous silver halide photographic emulsion is obtained.

#### References Cited

#### UNITED STATES PATENTS

|           |         |                |       |        |
|-----------|---------|----------------|-------|--------|
| 1,602,592 | 10/1926 | Sheppard       | ----- | 96—107 |
| 1,962,133 | 6/1934  | Brooker et al. | ----- | 96—109 |
| 3,148,276 | 9/1964  | Rothstein      | ----- | 250—65 |
| 3,189,458 | 6/1965  | Herz           | ----- | 96—108 |

NORMAN G. TORCHIN, Primary Examiner.

J. R. EVERETT, Assistant Examiner.

UNITED STATES PATENT OFFICE  
CERTIFICATE OF CORRECTION

Patent No. 3,411,917

November 19, 1968

John Figueras

It is certified that error appears in the above identified patent and that said Letters Patent are hereby corrected as shown below:

Column 1, line 31, after "sensitivity" cancel the comma. Column 2, line 58, "-2-(3H)-" should read -- -2(3H)- --. Column 4, line 9, "2,716,062, issued Aug. 23, 1955" should read -- 2,444,609, issued July 6, 1948 --.

Signed and sealed this 10th day of March 1970.

(SEAL)

Attest:

Edward M. Fletcher, Jr.

Attesting Officer

WILLIAM E. SCHUYLER, JR.

Commissioner of Patents